

Oct. 24, 1933.

E. M. FREELAND

1,932,307

SILICON STEEL AND METHOD OF MAKING THE SAME

Filed Sept. 13, 1932

3 Sheets-Sheet 1



**INVENTOR**

INVENTOR  
Edward M. Freeland  
by his attorneys

Bynes, Stubbins, Parmelee & Blenko

Oct. 24, 1933.

E. M. FREELAND

1,932,307

SILICON STEEL AND METHOD OF MAKING THE SAME

Filed Sept. 13, 1932

3 Sheets-Sheet 2



*Fig. 7.*



*Fig. 8.*



*Fig. 9.*



INVENTOR

Edward M. Freeland  
by his attorneys

Bynes, Stebbins, Parmelee & Blenko

Oct. 24, 1933.

E. M. FREELAND

1,932,307

SILICON STEEL AND METHOD OF MAKING THE SAME

Filed Sept. 13, 1932

3 Sheets-Sheet 3



Patented Oct. 24, 1933

1,932,307

# UNITED STATES PATENT OFFICE

1,932,307

## SILICON STEEL AND METHOD OF MAKING THE SAME

Edward M. Freeland, Youngstown, Ohio

Application September 13, 1932  
Serial No. 632,917

14 Claims. (Cl. 148—12)

The present invention relates broadly to the art of metal working, and more particularly to that branch of the art having to do with the subjecting of a predetermined composition or alloy to a treatment of such nature that the electrical properties thereof are materially modified, thereby enabling the production of an improved article having such properties as to better adapt it to electrical uses.

It is customary in order to improve the efficiency of different types of electrical apparatus, such as motors, dynamos, transformers and the like, to utilize a ferrous material, usually in the form of a series of sheets or laminae characterized by a high electrical efficiency from the standpoint of watt loss, magnetic permeability, low magnetic hysteresis and the like. In this connection, it is known that sheets of iron-silicon, or iron-silicon-aluminum alloys constitute a superior material. The present invention contemplates not only a variation in the silicon content for the purpose of obtaining certain desirable results, but also a special mechanical and heat treatment whereby the material with a given silicon content will have its electrical properties improved.

It is customary in the art to divide so-called electrical steels into a number of different grades, generally with reference to the particular use to which the steels are to be put. It is to be understood, therefore, that the term "electrical steels" or its equivalent, as hereinafter utilized, unless specifically restricted to a specified grade by way of example, is to be considered as a generic term including all the various grades without regard to the specific properties or uses contemplated.

For purposes of a better understanding of the invention, it will hereinafter be illustrated and described as applicable to a ferrous material containing silicon, having a low watt loss and produced initially from a hot rolled strip, the term "strip" being used herein in its commonly accepted sense in the steel industry.

Among other things, I have found that the efficiency of electrical steels, regardless of their grade, or silicon content, when intended for use as laminae in apparatus of the character described, is materially improved where the steel is produced by a method which includes an operation which will impart the smooth surface generally characteristic of a cold rolling operation, or an operation generally equivalent thereto. Such a smooth surface enables the individual sheets to be assembled in more compact relationship, thereby providing a greater metal cross section, and consequently, a greater magnetic flux

path, per unit of area. In this connection, however, it is desirable that where steels have such a surface characteristic, the treatment include as one of the steps thereof a heat treating operation under such conditions as to insure a film of oxidized metal on the surface of the steels. Such a film, where closely adhering and of relatively minute thickness, provided an insulating layer between adjacent laminae in such manner that the disadvantages, such as objectionable heating, which usually characterize laminae free of any insulation, or a solid core, are obviated.

As a general observation, it may be stated that the electrical properties, particularly with respect to watt loss, are improved as the silicon content is increased. I have likewise found that regardless of the silicon content, provided it lies within a certain range, the electrical properties may be improved by certain characteristic treatment steps preferably in a certain order. There are thus afforded two variables which must be taken into consideration in the production of any given grade of material, it being possible with a relatively lower silicon content to obtain the desired results by a more elaborate mechanical and/or heat treating operation, or with a relatively higher silicon content to obtain the desired results utilizing a relatively simpler and usually fewer number of mechanical and heat treating steps. As to certain grades, however, wherein best guarantees, particularly with respect to watt loss, must be met, it is necessary to resort not only to the advantages incident to a relatively higher silicon content, but also to the most advantageous series and sequence of heat treating and mechanical treatment steps.

I have also found that the electrical properties of a steel of the character herein contemplated are improved materially when the steel is produced by a rolling operation characterized throughout by rolling in the direction only in which the original ingot was reduced in the blooming mill, provided the user of the material takes advantage of the direction of rolling and so cuts and assembles the laminae that in the completed structure the direction of the magnetic flux will be parallel or substantially parallel to the direction of rolling. My invention therefore contemplates, among other things, a material which, regardless of its silicon content and the different treatment steps to which it may have been subjected, will be characterized by having been subjected to rolling in one direction only.

Reference has heretofore been made to the fact that the invention preferably contemplates the

production of electrical steels from material which at least at some time during the treatment to which it is subjected has been in the form of a hot rolled strip. Heretofore, the only 5 known method of reducing a hot rolled strip to certain of the gauges required for electrical steels, has been by cold rolling, and it has been a commonly accepted belief that the excessive strain incident to the cold rolling operation would pre- 10 clude the use of such a material from the electrical field. My invention not only provides a method of treatment wherein the objections incident to such excessive strain may be completely obviated, but whereby the material when delivered in the 15 form of a one-piece strip wound in successive convolutions to provide a coil to facilitate handling and transportation thereof, may be substantially free from coil set. Elimination of coil set, from a coiled strip of electrical steel which, 20 in itself, constitutes a new article of manufacture, enables laminae to be cut from the metal of the coil and assembled without introducing strain in the laminae by the flattening operation usually incident to the assembly of the laminae.

25 The production of the hot rolled strip which is used in the present invention may be effected by suitable hot rolling in a succession of passes to a desired gauge while always rolling the metal in the direction only in which the ingot was rolled. 30 Such a succession of passes may obviously be obtained by repeatedly subjecting the metal to rolling operations in the same mill, or to repeated rolling operations in a succession of mill stands such as afforded by a continuous or tandem mill. 35 While the last mentioned procedure is desirable from the standpoint of production and the comparatively few handling operations involved, it will be apparent to those skilled in the art that my invention is not limited to the constructional 40 or operating characteristics of the mills, or the number of stands utilized in perfecting the production of the hot rolled strip. It is desirable, in accordance with my invention, that the last hot rolling operation be accomplished at a temperature 45 which bears a definite and predetermined relationship to the recalescence point of the particular material undergoing treatment. If the material, during the last hot rolling pass, is at a temperature higher than the recalescence 50 temperature, the finished material, with a given silicon content, will be characterized by an absence of re-crystallization and by certain electrical properties. If the last rolling operation in the hot mill is accomplished at substantially the 55 recalescence temperature, the material while characterized likewise by the absence of re-crystallization will have generally superior electrical properties to the product before referred to. In like manner, final rolling at a temperature 60 slightly below the recalescence temperature will further improve the electrical properties. While such material may be characterized by grain growth, I have found that at least insofar as it has been possible to make any definite measurements, the grain growth is not a determining factor in the electrical characteristics. If the last 65 hot rolling step is accomplished at a temperature sufficiently below the recalescence point to cause re-crystallization upon subsequent heat treatment, the resulting product will have electrical properties which are generally inferior to the corresponding properties characteristic of material wherein the last hot rolling was at a temperature above, equal to, or but slightly below 70 the recalescence point. By properly varying the

silicon content, however, a material rolled with the last pass appreciably below the recalescence point may have electrical properties superior to metal of a lower silicon content rolled at slightly below or above the recalescence point.

80 In most cases, it has been proposed in the art to subject silicon steel in sheet form to an annealing operation. While such an annealing operation may be utilized in accordance with my invention, I have found that the properties desirable from an electrical standpoint are improved if normalizing is practiced on the material instead of annealing, and that these properties may be further improved by an operation including both normalizing and annealing, generally regardless of the order in which these two heat treating steps are performed. I am therefore of the belief that the electrical properties for some reason unknown to me vary in proportion to the temperature to which the material, regardless of how produced, is subjected.

85 From the foregoing it will be apparent that apart from the rolling in one direction only, and special treatment steps which will be hereinafter described, there are three variables which must be taken into account in the production of electrical steel to meet the guarantees for a required grade, these variables being, respectively, and probably in the order of importance, the silicon content, the temperature at which the last hot 90 rolling pass is accomplished, and the temperature at which the heat treating following the hot rolling is carried out.

95 In the accompanying drawings, I have shown, largely diagrammatically, for purposes of illustration only, certain practices in accordance with which my invention may be carried out. In the drawings, Figures 1 to 15, inclusive, are diagrammatic views illustrating different characteristic operations both as to sequence and type, each 100 operation, however, being characterized by a rolling of the material throughout in the direction only in which the material is reduced from the ingot in the blooming mill. In all of the figures, I have used descriptive legends for the purpose of facilitating a reading and understanding of the operations diagrammatically illustrated.

105 In accordance with the form of my invention illustrated in Figure 1, a suitable silicon steel ingot having the desired silicon content is subjected to the usual back and forth rough rolling in the blooming mill 2 for reducing it to a billet 3. This billet in turn may be subjected to suitable hot rolling in a succession of passes in a hot mill herein illustrated as comprising four 110 roll stands 4 effective for producing a hot rolled strip 5. This hot rolled strip may be subjected to a suitable pickling operation in a pickling bath 6, effective for producing a pickled hot 115 rolled strip 7. This hot rolled strip may then be heated in any suitable furnace 8 up to a temperature bearing a predetermined relationship to the recalescence temperature of the metal and previously determined upon by reason of the 120 silicon content and the grade of steel to be produced. Having been raised to this temperature, it may be given a final pass in a hot roll stand 9 effective for producing a hot rolled strip 10. This strip may then be coiled in a suitable coiler 11 and 125 annealed in a suitable box annealing chamber 12. If desired, the box annealing may be replaced by normalizing. In the case of a box anneal, the product may be sold directly, or it may be reheated and allowed to cool in the flat to re- 130

135

140

145

150

155

160

165

170

175

180

185

190

195

200

move coil set. In the case of normalizing, the product may be immediately coiled, or it may be allowed to cool in the flat before coiling, in order to preclude any coil set. This latter procedure will be more clearly pointed out in connection with Figure 5. Also it will be apparent that the box anneal or normalized product so produced may be subjected to a suitable leveling operation, as by a roller leveller, then sheared and either box annealed or normalized.

In the showing of Figure 1, the roll stands 4 may be considered as only effective for rolling to an intermediate gauge, and the stand 9 effective for producing the finished gauge.

In Figure 1, I have indicated the heating furnace 8, the hot roll stand 9 and the hot rolled strip 10 as included within a frame bearing the designation "May omit under specified conditions". Thus, if the rolling operation in the hot mill including the stands of rolls 4, is so carried out that the last hot rolling operation is at the desired predetermined temperature with relationship to the recalescence temperature, it is unnecessary to effect subsequent heating of this material to such a temperature followed by rolling. In most cases, however, an accurate temperature control without heating is difficult, so that a heating furnace in advance of the last rolling pass may usually be considered as desirable. To this end, I may, if desired, locate the heating furnace 8 in the dotted line position 18 of Figure 1 wherein it will be effective for insuring the last hot rolling pass at the desired temperature, and then eliminate the hot roll stand 9.

In Figure 2 there is illustrated a slightly modified embodiment of the invention wherein parts corresponding to the parts shown in Figure 1 are designated by the same reference characters having the suffix *a* added thereto. In accordance with this embodiment, the pickled hot rolled strip 7*a* is sheared by a suitable shear 14 to provide a plurality of pieces of sheared hot roll strip 15. These individual pieces 15 may then be raised to the predetermined temperature in the heating furnace 8*a*, hot rolled at that temperature in the roll stand 9*a* to provide sheets 16, which are then box annealed or normalized in a suitable furnace or box 17. If desired, there may be both an anneal and normalizing. With this form of the invention, assuming that the furnace 18*a* has been utilized, the parts 8*a*, 9*a* and 16 enclosed within the border may be omitted for reasons pointed out in connection with Figure 1. It will also be apparent that the shear 14 can be placed after the furnace on box 17, and then followed by a normalizing or annealing treatment.

In Figure 3, parts corresponding to the parts illustrated in Figure 2 are designated by the same base number with the suffix *b* added thereto. In accordance with this form of my invention, sheets after having been box annealed or normalized in the furnace or box 17*b*, are subjected to a cold rolling operation in a roll stand 21, preferably so adjusted as to introduce a strain in the sheets corresponding to that represented by an elongation of somewhere in the range of from approximately 1 to 5%. While an elongation of 1% will introduce sufficient strain for the purposes intended, I have found that the introduction of additional strain up to the limit indicated is not objectionable and constitutes a safety factor in insuring that at least the desired minimum will be introduced. The strained sheets 22 having this desirable strain component therein are then subjected to an annealing or normalizing

operation, preferably in a suitable furnace or box 23. I have found that such a strain introduction followed by a heat treating operation, which may be in the form of a box anneal and preferably at a temperature in excess of 1600°, gives a material having electrical properties which are superior to a material similarly produced and with a similar silicon content, but which has not had such a strain introduced and subsequently removed therefrom.

In Figure 4, there is illustrated another embodiment of my invention in which parts corresponding to the parts illustrated in Figure 1 are designated by the same reference characters having the suffix *c* added thereto. In accordance with this embodiment of the invention, the coiled strip after having been subjected to a box annealing or normalizing 12*c* is given a cold rolling treatment in one or more cold rolling stands 21*c*, corresponding in function to the stand 21 of Figure 3, but effective for producing a strip 24 having a desirable strain component of the character indicated therein. This strip may then be coiled in a suitable coiler 25 after which it may be placed in an annealing box 26 and 100 subjected to an annealing temperature of the order indicated for effecting substantially complete strain removal, or may be normalized for this purpose. In either case, coil set may be eliminated as referred to in connection with Figure 1.

In Figure 5, I have shown another embodiment of my invention which is generally similar to that illustrated in Figure 1, and wherein parts corresponding to the parts of Figure 1 are designated by the same reference characters having the suffix *d* added thereto. In accordance with this embodiment, the hot rolled strip after having been coiled in the coiler 11*d* is subjected to a normalizing treatment in a normalizing furnace 115 27, after which it may be again coiled in a suitable coiler 28. By the normalizing operation, the material is subjected to a higher temperature than that which is generally considered possible of attainment by annealing and more particularly box annealing, and the electrical properties are correspondingly improved. This modification has been referred to in connection with Figure 1, as well also as the possibility of placing a shear after the furnace 28, followed by further heat treatment, if desired. By spacing the coiler 28 from the furnace 27, the material may be cooled in the flat before coiling and coil set obviated.

Figure 6 shows an embodiment generally similar to Figure 5, with the parts designated by the same reference characters as those used in Figure 1, but with the suffix *e* added thereto. In accordance with this form, a strip coiled in the coiler 11*e* is passed through either a normalizing or an annealing furnace 29 and either normalized or annealed, and thereafter passed through an annealing or normalizing furnace 30, wherein the operation which was not performed in the furnace 29 is carried out. Thereafter, the material in strip form which has been subjected to both an annealing and normalizing operation is coiled in a suitable coiler 28*e*. Suitable shearing and heat treating may follow the unit 20, or the treatment may be as before described, to remove or prevent coil set.

Attention has already been called to the fact that the step of strain introduction followed by a proper heat treating operation improves the electrical properties. In Figure 7, there is shown a lay-out generally similar to that of Figure 5, 150

but differing therefrom in that the normalized material either before or after coiling in the coiler 28f is subjected to cold rolling in a roll stand 21f, effective for introducing a desirable 5 strain component therein. Thereafter the material may be passed directly into a normalizing furnace 30f, or may be first coiled in a suitable coiler 31 and thereafter given a box anneal in the annealing chamber 30f. If subjected to normalizing, it may be coiled after the normalizing 10 operation in a suitable coiler 32. If the unit 30 serves to anneal, the annealed coil may be reheated and then cooled in the flat before coiling.

The lay-out of Figure 8 is similar to that of 15 Figure 7, and the same system of reference numerals has been followed with the suffix changed. In accordance with this embodiment, the material after having been subjected to strain introduction in the cold rolling stand 21g and 20 either before or after having been coiled in a suitable coiler 31g is subjected to normalizing in a furnace 30g. Upon leaving the furnace it is carried an appreciable distance in flat form, and permitted to cool in this form so as to remove coil set, after which it is coiled in a suitable coiler 32g. In this manner, there is obtained a material which, when unwound from the coil, will lie perfectly flat with the result that 25 the laminae cut or punched therefrom will also lie flat and thus permit of assembly without the 30 introduction of a flattening strain. In this manner, a superior product is insured.

With the forms of my invention heretofore described and particularly those illustrated in 35 Figures 3, 4, 7 and 8, the strain introduction involves only a very small reduction in thickness, and while relied upon to give some reduction, is primarily for the purpose of introducing a desirable strain component of the order referred to. 40 In many cases, however, the hot rolling operation and particularly where carried out in a continuous mill is customarily relied upon for producing a hot rolled strip substantially free from any cold working strains, having a thickness of 45 approximately .0625 inch, corresponding to 16 gauge, and having any desired width. Electrical sheets customarily have a thickness lying within and including 22 to 30 gauge (United States standard). This material in strip form can most 50 effectively be reduced by cold rolling in a continuous mill, but such a continuous mill has heretofore been considered impracticable for the production of electrical steels by reason of the excessive strain introduced into the metal thereby, 55 the cold rolling effecting a very appreciable reduction. If this reduction is from .0625 inch to .024 inch, there is a reduction of .0385 inch, equal to approximately 61%. These figures are 60 representative of thicknesses frequently produced in the cold rolling of steel for purposes other than the production of electrical steels. While such a cold rolling operation is effective for reducing the hot rolled strip to the desired finished gauge, the strain introduced by reason of the reduction 65 effected is far in excess of the strain heretofore though permissible in the production of electrical steels. In accordance with one embodiment of my invention, however, I take advantage of the strain introduction thus effected, and consider 70 the strain as including both a desirable component of the order previously mentioned and an undesirable component, which is that in excess of the desirable component. In Figure 9, I have shown an embodiment of the invention operating 75 according to the immediately preceding description.

In this form of the invention, material, for example, after having been normalized or annealed at 27h and after being coiled in a suitable coiler 28h, is passed to a continuous cold mill 33 comprising a plurality of stands in tandem effective for giving the desired reduction in thickness. As an incident to this reduction, the excessive strain referred to is introduced. This material may then be coiled in a coiler 34 and subjected to a partial annealing in a suitable furnace 35 after which it may or may not be coiled in a suitable coiler 36 and then subjected to a normalizing operation in a furnace 37, after which it may be coiled for shipment in a suitable coiler 38. On the other hand, after leaving the coiler 34, it may be partially normalized in the furnace 35 and then, after coiling in the coiler 36, be annealed in the furnace 37, or without such coiling or with it as preferred, be normalized in this furnace. If normalized it may again be coiled in the coiler 38. 80 85 90 95

In my copending application Ser. No. 593,783, filed February 18, 1932, I have described and claimed the general two-stage heat treating operation including a partial anneal or a partial 100 normalizing followed either by a complete anneal or a complete normalizing, the partial anneal or partial normalizing being carried out to the extent required to remove the undesirable strain component and leave only the desirable 105 strain component in the material, so that the final anneal or normalize will be effective on material which only has such a desirable strain component therein.

With any given silicon content, the undesirable strain component will vary with changes in the reduction effected by the cold rolling operation, the strain increasing with increased reductions, and decreasing with smaller reductions. While the actual strain introduced under varying reductions is not a straight line function, it is a function which is readily determinable.

In like manner, the undesirable strain component increases in amount as the silicon content of the material undergoing treatment increases, with any given percentage of reduction by the cold mill. 110 115 120

In practicing my invention I have successfully employed a continuous heating furnace as indicated at 35 in Figure 9. The furnace had a 125 length of approximately 30 feet and was maintained at a temperature of approximately 1900° F. Silicon steel strip containing approximately 1% of silicon, which steel had been subjected to a 61% reduction by cold rolling, and having a 130 final thickness of .024", was passed through the furnace at the rate of 15 feet per minute, giving a total time in the furnace of two minutes. I have estimated that in the furnace employed the heat penetrated with sufficient rapidity to 135 bring the strip up to the desired minimum temperature in approximately 30 seconds, thus leaving 90 seconds of additional heating time available for continued heating. Under the above conditions the heat treatment eliminated the 140 undesirable strain component and left the desirable strain component therein.

It is generally assumed that the rate of heat penetration varies directly with the thickness of the material and hence if the strip being treated were only half as thick, that is to say, .0125 inches, then only 15 seconds would be required to bring it up to the desired minimum temperature. Adding to this the continued heating time of 90 seconds, the total time for heating 145 150

such strip in the furnace in question would be 105 seconds.

It may thus be ascertained that the total time-temperature treatment for effecting removal of the undesirable strain component varies directly as the thickness of the material undergoing treatment, assuming a predetermined silicon content and a predetermined reduction. This treatment may be considered as involving the two factors of time and temperature. If it is desired to decrease the time of treatment, it is necessary to increase the temperature, while if it is desired to increase the time, there should be a corresponding reduction in temperature.

Since the undesirable strain component increases with higher silicon and decreases with lower silicon, and likewise increases with the percentage of reduction and vice versa, it is necessary to make a corresponding change in the time-temperature characteristic to accommodate the treatment to either the silicon content or the percentage of reduction. By taking these factors into consideration, the furnace 35, whether an annealing or a normalizing furnace, may be used for partial strain removal only, with definite assurance that a desirable strain will be retained in the material.

Figure 10 illustrates an operation generally similar to that of Figure 9, but differing in that the material coiled in the coiler 38<sup>l</sup> is heated in a suitable furnace 39 and then cooled in the flat to remove coil set before being subsequently coiled in the coiler 32<sup>l</sup>.

In Figure 11, the material after having been cold rolled in the continuous mill 33<sup>j</sup> and after having been coiled in the collar 34<sup>j</sup> may be either annealed or normalized in a furnace 40. Thereafter it may be coiled in a coiler 41, passed through a cold rolling stand 21<sup>j</sup> effective for introducing a desirable strain component only, thereafter recoiled in a coiler 42 with subsequent annealing or normalizing in a furnace 37<sup>j</sup> followed by coiling in a collar 38<sup>j</sup>. With this form of the invention, it will be apparent that the heat treating furnace 40 is effective for completely removing all of the strain introduced by cold rolling, and that thereafter, only a desirable strain component is introduced.

Figure 12 shows a lay-out generally similar to that of Figure 9, but differing principally in that the material, usually after having been coiled in a coiler 36<sup>k</sup>, is passed through a normalizing furnace 43 and thereafter cooled in the flat to remove coil set and then coiled in a suitable coiler 32<sup>k</sup>.

In Figure 13, the operations correspond generally to those carried out in accordance with Figure 11, up to the point of coiling in the coiler 42<sup>l</sup>. After this operation, the material is normalized in a furnace 43<sup>l</sup>, cooled in the flat to remove coil set and coiled in the coiler 32<sup>l</sup>.

The next two figures of the drawings differ from each other in that one relates to excessive strain introduction and the other to normal strain introduction only. The procedure in accordance with Figure 14 is generally similar to that of Figure 7, up to the coiler 31<sup>m</sup>. From this coiler, the

material may pass through a roller leveler 44 to a suitable shear 14<sup>m</sup> effective for producing sheets 45 which may thereafter be box annealed in an annealing box 19<sup>m</sup>.

In Figure 15, the operation of Figure 9 is followed up to the coiling in the coiler 34<sup>n</sup> after which the material may pass through a roller leveler 44<sup>n</sup> to a shear 14<sup>n</sup> effective for forming sheets 45<sup>n</sup> which may be partially annealed in a box 46 to remove only the undesirable strain component and thereafter again anneal in a suitable box anneal 47 to complete the strain removal.

If in any case, the finishing temperature on the hot mill, where rolling to an intermediate gauge, is not satisfactorily controlled, an annealing or normalizing step may be introduced following the hot rolling to intermediate gauge and prior to any subsequent rolling.

The pickling step illustrated may be varied as to its time of performance, as desired, its function being only to effect removal of scale or oxide.

Also, the shearing step may be practiced without roller leveling, if desired, although I have found the leveling operation to be generally more satisfactory.

Wherever the material is annealed in coils, it may be reheated and cooled in the flat to remove coil set, and wherever it is normalized in strip form, it may be cooled in the flat before being recoiled, in order that coil set may be eliminated.

From the foregoing description, it will be apparent that all forms of my invention contemplate starting with a hot rolled strip followed by certain after operations, including in some cases limited cold rolling and in other cases material reduction by cold rolling. In all cases, any rolling is in the direction of the original rolling operation in the roughing mill or, to be more specific, the material at no time is subjected to a cross rolling operation. This constitutes one of the features of my invention.

Another feature of my invention relates to the accomplishing of the last hot rolling pass in definite predetermined relationship to the recalcence point of the metal for reasons pointed out in detail.

My invention further contemplates taking advantage of the variable factors hereinbefore referred to and using them either individually or combined to produce superior electrical properties. By properly utilizing these variables, it is possible to meet guarantees as shown below in the table containing seven different grades of electrical steels, each with an identifying title, together with the watt loss per pound at frequencies of both 50 and 60 cycles at the assumed specific gravities indicated, the maximum watt losses in the case of some of the grades being shown for a plurality of different gauges, these ranges covering the gauges ordinarily manufactured. In all cases, the watt loss is figured at a flux density of 10,000—B and determined in accordance with the specification A—34—28 of the American Society for Testing Materials. There is indicated one permissible range of silicon variation for each grade.

Regular transformer (Assumed sp. gr. 7.50)  
Silicon 3% plus—U. S. standard gauges

| 70                           | 30 G. | 29 G. | 28 G. | 27 G. | 26 G. | 25 G. | 24 G. | 23 G. | 22 G. | 145 |
|------------------------------|-------|-------|-------|-------|-------|-------|-------|-------|-------|-----|
| Watts per lb.—60 cycles..... | .76   | .76   | .80   | .85   | .89   | .93   | .98   | ..... | ..... |     |
| Watts per kg.—60 cycles..... | 1.67  | 1.67  | 1.76  | 1.87  | 1.96  | 2.05  | 2.16  | ..... | ..... |     |
| Watts per lb.—50 cycles..... | .62   | .62   | .64   | .68   | .71   | .75   | .78   | ..... | ..... |     |
| Watts per kg.—50 cycles..... | 1.375 | 1.375 | 1.41  | 1.50  | 1.56  | 1.65  | 1.72  | ..... | ..... |     |

Special transformer (Assumed sp. gr. 7.50)  
Silicon 3% plus

|    | 30 G.                                                                             | 29 G. | 28 G. | 27 G. | 26 G. | 25 G. | 24 G. | 23 G. | 22 G. |      |
|----|-----------------------------------------------------------------------------------|-------|-------|-------|-------|-------|-------|-------|-------|------|
| 5  |                                                                                   |       |       |       |       |       |       |       |       | 30   |
|    | Watts per lb.—60 cycles.....                                                      |       | .70   |       |       |       |       |       |       |      |
|    | Watts per kg.—60 cycles.....                                                      |       | 1.54  |       |       |       |       |       |       |      |
|    | Watts per lb.—50 cycles.....                                                      |       | .56   |       |       |       |       |       |       |      |
|    | Watts per kg.—50 cycles.....                                                      |       | 1.24  |       |       |       |       |       |       |      |
| 10 | Extra special transformer (Assumed sp. gr. 7.50)<br>Silicon 3% plus               |       |       |       |       |       |       |       |       | 85   |
| 15 | Watts per lb.—60 cycles.....                                                      |       | .64   |       |       |       |       |       |       |      |
|    | Watts per kg.—60 cycles.....                                                      |       | 1.42  |       |       |       |       |       |       |      |
|    | Watts per lb.—50 cycles.....                                                      |       | .52   |       |       |       |       |       |       |      |
|    | Watts per kg.—50 cycles.....                                                      |       | 1.15  |       |       |       |       |       |       |      |
|    | Armature (Assumed sp. gr. 7.70)<br>Silicon .3-.7 (U. S. standard gauges)          |       |       |       |       |       |       |       |       |      |
| 20 | Watts per lb.—60 cycles.....                                                      | 1.35  | 1.40  | 1.46  | 1.53  | 1.65  | 1.85  | 2.15  | 2.50  | 2.80 |
|    | Watts per kg.—60 cycles.....                                                      | 2.97  | 3.08  | 3.20  | 3.57  | 3.63  | 4.07  | 4.73  | 5.50  | 6.16 |
|    | Watts per lb.—50 cycles.....                                                      | 1.12  | 1.17  | 1.20  | 1.30  | 1.42  | 1.53  | 1.75  | 2.00  | 2.30 |
|    | Watts per kg.—50 cycles.....                                                      | 2.46  | 2.57  | 2.64  | 2.86  | 3.12  | 3.57  | 3.85  | 4.40  | 5.06 |
| 25 | Electrical (Assumed sp. gr. 7.70)<br>Silicon .75-1.5 (U. S. standard gauges)      |       |       |       |       |       |       |       |       | 100  |
| 30 | Watts per lb.—60 cycles.....                                                      | 1.15  | 1.20  | 1.28  | 1.35  | 1.40  | 1.55  | 1.80  | 2.10  | 2.30 |
|    | Watts per kg.—60 cycles.....                                                      | 2.53  | 2.64  | 2.82  | 2.97  | 3.08  | 3.41  | 3.96  | 4.62  | 5.06 |
|    | Watts per lb.—50 cycles.....                                                      | .95   | 1.00  | 1.07  | 1.14  | 1.18  | 1.30  | 1.50  | 1.70  | 1.85 |
|    | Watts per kg.—50 cycles.....                                                      | 2.09  | 2.20  | 2.35  | 2.51  | 2.60  | 2.86  | 3.30  | 3.74  | 4.07 |
|    | Special motor (Assumed sp. gr. 7.50)<br>Silicon 2.0-3.0 (U. S. standard gauges)   |       |       |       |       |       |       |       |       | 105  |
| 35 | Watts per lb.—60 cycles.....                                                      | 1.00  | 1.03  | 1.08  | 1.15  | 1.20  | 1.25  | 1.30  |       |      |
|    | Watts per kg.—60 cycles.....                                                      | 2.20  | 2.27  | 2.38  | 2.53  | 2.64  | 2.75  | 2.86  |       |      |
|    | Watts per lb.—50 cycles.....                                                      | .84   | .86   | .90   | .94   | .97   | 1.00  | 1.05  |       |      |
|    | Watts per kg.—50 cycles.....                                                      | 1.85  | 1.89  | 1.98  | 2.07  | 2.13  | 2.20  | 2.31  |       |      |
| 40 | Special dynamo (Assumed sp. gr. 7.50)<br>Silicon 2.75-3.5 (U. S. standard gauges) |       |       |       |       |       |       |       |       | 115  |
| 45 | Watts per lb.—60 cycles.....                                                      | .85   | .86   | .90   | .95   | 1.00  | 1.05  | 1.10  |       |      |
|    | Watts per kg.—60 cycles.....                                                      | 1.87  | 1.89  | 1.98  | 2.09  | 2.20  | 2.31  | 2.42  |       |      |
|    | Watts per lb.—50 cycles.....                                                      | .68   | .70   | .73   | .77   | .82   | .88   | .90   |       |      |
|    | Watts per kg.—50 cycles.....                                                      | 1.50  | 1.55  | 1.61  | 1.70  | 1.81  | 1.89  | 1.98  |       |      |

40 My invention further contemplates the production of superior electrical steel in either sheet or coil form, and in the case of coil strip either with or without the coil set removed therefrom.

50 Other advantages of the invention will be readily apparent to those skilled in the art from the foregoing descriptions and illustrations, it being understood that changes in the construction and relationship of the parts may be made 55 without departing either from the spirit of my invention or the scope of the broader claims, the figures of the drawings being illustrative only and not exclusive of various changes, such, for example, as generally referred to herein.

60 I claim:

65 1. In the method of making silicon steel in sheet-like form, the steps consisting in casting a steel ingot of the desired silicon content and hot rolling the ingot to reduce it, all the hot rolling passes in which any substantial reduction is effected being in the direction in which the ingot was rolled, thereby to improve the electrical properties of the material.

70 2. In the method of making silicon steel in sheet-like form, the steps consisting in casting a steel ingot of the desired silicon content and hot rolling the ingot to reduce it, all the hot rolling passes in which any substantial reduction is effected being in the direction in which the ingot

was rolled, thereby to improve the electrical properties of the material, and further controlling the electrical properties of the steel by varying the temperature at which the last hot rolling is effected.

3. In the method of making silicon steel in sheet-like form, the steps consisting in casting a steel ingot of the desired silicon content, hot rolling the ingot to reduce it, all the hot rolling passes in which any substantial reduction is effected being in the direction in which the ingot was rolled, thereby to improve the electrical properties of the material, and then raising the temperature of the material sufficiently to effect substantial elimination of the strains therein.

4. In the method of making silicon steel in sheet-like form, the steps consisting in casting a steel ingot of the desired silicon content, hot rolling the ingot to reduce it, all the hot rolling passes in which any substantial reduction is effected being in the direction in which the ingot was rolled, thereby to improve the electrical properties of the material, raising the temperature of the material sufficiently to effect elimination of part but not all of the strains therein, allowing the material to cool, and then annealing it.

5. In the method of making silicon steel in sheet-like form, the steps consisting in casting a steel ingot of the desired silicon content, hot roll-

- ing the ingot to reduce it, all the hot rolling passes in which any substantial reduction is effected being in the direction in which the ingot was rolled, thereby to improve the electrical properties of the material, then raising the temperature of the material sufficiently to effect substantial elimination of the strains therein, then so working the material as to introduce strain therein, and then annealing it to remove such strain. 5
- 10 6. In the method of making silicon steel in sheet-like form, the steps consisting in casting a steel ingot of the desired silicon content, hot rolling the ingot to reduce it, all the hot rolling passes in which any substantial reduction is effected being in the direction in which the ingot was rolled, thereby to improve the electrical properties of the material, then raising the temperature of the material sufficiently to effect substantial elimination of the strains therein, cold rolling the material, 15 and then annealing it. 20
7. As a new article of manufacture, electrical steel in sheet-like form containing .1 to 6% silicon and having the electrical properties characteristic of those obtained when a steel of substantially the same silicon content within such range is subjected to reduction by hot rolling with all substantial reductions effected by rolling in the same direction. 25
8. As a new article of manufacture, electrical steel in sheet-like form containing .1 to 6% silicon and having the electrical properties characteristic of those obtained when a steel of substantially the same silicon content within such range is subjected to reduction by hot rolling with all substantial reductions effected by rolling in the same direction, followed by heating to a temperature sufficient to remove the strain. 30
9. As a new article of manufacture, electrical steel in sheet-like form containing .1 to 6% silicon and having the electrical properties characteristic of those obtained when a steel of substantially the same silicon content within such range is subjected to reduction by hot rolling with all substantial reductions effected by rolling in the same direction, followed by heating to a temperature sufficient to remove the strain, cold rolling to effect a substantial reduction in thickness, and annealing. 35
- 40 10. As a new article of manufacture, electrical steel in sheet-like form containing .1 to 6% silicon and having electrical properties characteristic of those obtained when a steel of sub-
- stantially the same silicon content within such range is subjected to reduction by hot rolling with all substantial reductions effected by rolling in the same direction, followed by cold rolling to effect a substantial reduction in thickness, heating to a sufficient temperature and for such limited time as to remove part but not all of the strain in the material, cooling and then annealing it, all substantial reductions which are made being effected by rolling in the same direction. 45
11. In the method of making silicon steel in sheet-like form, the steps consisting in casting a steel ingot of the desired silicon content and reducing the ingot to sheet-like form by hot rolling passes and subsequent cold rolling passes, all of the rolling passes in which any substantial reduction is effected being in the direction in which the ingot was rolled, thereby to improve the electrical properties of the material. 50
12. As a new article of manufacture, electrical steel in sheet-like form containing .1 to 6% silicon and having the electrical properties characteristic of those obtained when a steel of substantially the same silicon content, within such range, is subjected to reduction by hot rolling passes followed by cold rolling passes, with all substantial reduction effected by rolling in the same direction. 55
13. As a new article of manufacture, electrical steel in sheet-like form containing .1 to 6% silicon and having the electrical properties characteristic of those obtained when a steel of substantially the same silicon content, within such range, is subjected to reduction by hot rolling followed by heating to a temperature sufficient to remove the strain, cold rolling to effect a substantial reduction in thickness, and annealing, all substantial reductions which are made being effected by rolling in the same direction. 60
14. As a new article of manufacture, electrical steel in sheet-like form containing .1 to 6% silicon and having electrical properties characteristic of those obtained when a steel of substantially the same silicon content, within such range, is subjected to reduction by hot rolling followed by cold rolling to effect a substantial reduction in thickness, heating to a sufficient temperature and for such limited time as to remove part but not all of the strain in the material, cooling, and then annealing it, all substantial reductions which are made being effected by rolling in the same direction. 65

EDWARD M. FREELAND.